

Jan. 18, 1927.

1,614,562

C. A. LAISE

APPARATUS AND METHOD OF WIRE DRAWING AND ALLOY WIRES USED  
FOR RADIOTUBES AND OTHER PURPOSES

Filed Sept. 5, 1925



WITNESS

Oliver W. Holmes

INVENTOR  
C. A. LAISE

BY  
Cornelia P. Billings  
his ATTORNEY

## UNITED STATES PATENT OFFICE.

CLEMENS A. LAISE, OF HAWORTH, NEW JERSEY.

## APPARATUS AND METHOD OF WIRE DRAWING AND ALLOY WIRES USED FOR RADIO-TUBES AND OTHER PURPOSES.

Application filed September 5, 1925. Serial No. 54,628.

My invention relates generally to an apparatus and process of manufacturing very fine wires of various metals or alloys of metals, and it is particularly adapted for the manufacture of very fine nickel-chromium alloy wires or tungsten alloy wires or molybdenum alloy wires particularly adapted for use as resistance wire, and in radiotubes, and other purposes.

10 It is well known in the art that very fine wires of certain metals or alloys cannot be drawn down by the ordinary processes of wire drawing after they reach a certain cross section because they lack sufficient tensile strength. It is also well known that tungsten and molybdenum wires when alloyed to a substantial degree with other metals or mixed with rare earths in a substantial amount cannot be mechanically worked and 20 drawn down to very fine size by the prior well known means and methods of the art and because also of a loss in the necessary tensile strength, and because also of the difficulty of obtaining suitable wire drawing dies, which 25 have the required fineness and which will retain their diameters during the drawing operation. The addition of a very small proportion of the rare earths to tungsten or molybdenum necessary to permit the use of the 30 resulting wires as filaments for incandescent lamps when operated on alternating current does not weaken the wire sufficiently to prevent wire drawing down to a small diameter by the processes of the prior art, but 35 when these additions or alloys are made to the greater degree which is required for use in radio tubes, then the product is so changed in its structure that it is weakened to such a degree that it does not have sufficient tensile strength in relation to its coefficient of friction to permit of its reduction in drawing by the mechanical working and the wire drawing of the ordinary 40 working and wire drawing processes now 45 known in the art.

The apparatus and process developed by me and which will be hereinafter described enables one to reduce the cross section of wires substantially uniformly throughout 50 their length after they have reached a size when their tensile strength no longer permits them to be drawn through dies by the well known processes of the prior art. In order to accomplish this important and necessary result, resort is had to electro-chemi-

cal means and in that, fundamentally, my invention consists. Through the combined action, therefore, of electrolysis and chemical solution upon the material of the wire when the wire is passing through a suitable bath of electrolyte one is enabled to uniformly reduce the cross section of a metal wire which could not be drawn further down by the ordinary processes of wire drawing and thus the wire products are made suitable for uses in the art to which they could not have heretofore been put because of the fact that the art had not disclosed a method to accomplish those ends.

It is well known, of course, that a chemical solution has heretofore been resorted to and electro-chemical processes have been resorted to for the purpose of cleaning and pointing wires or sharpening instruments, but I believe that I am the first to utilize these agents for the actual manufacture of very fine wires for useful and particularly for commercial purposes. I thus produce very fine wires having roughened surfaces which I have found to be much superior for radio tube filament to wires of the same size having a smooth surface as a wire having a smooth surface does not give as high an electron emission as does the same size wire having a roughened surface. Since, therefore, by my process of reducing the diameter of the wire by electro-chemical means produces a wire with a roughened surface, I thereby produce a superior wire of higher electron emission than any heretofore produced.

By the term roughened surface, I mean a surface which is not polished which is the inevitable result of the ordinary method of wire drawing now known in the art.

In the manufacture of wires for radio tubes capable of high electron emission it is customary to use as an ingredient of these wires the metals tungsten, molybdenum, platinum, and so forth. It is necessary however to activate these metals by the addition thereto or the alloying therewith of substantial amounts of either thorium, yttrium, vanadium, strontium, barium compounds, etc. As soon, however, as the above elements in the substantial amounts required for radio work have been added to or alloyed with the pure metals of tungsten, molybdenum or platinum, it is difficult, as has been said above, if not actually impossible, to pro-

duce the resultant composite wire having a sufficient fineness of cross section by the ordinary metal working processes of whatever nature.

5 It is a fact that in many cases excellent compositions capable of high electron emission have had to be discarded because their tensile strength and physical condition would not permit them to be drawn down to 10 a size so they could be used in either power tubes or radio tubes.

The operation of my process may be carried out in the apparatus which I have illustrated conventionally in the drawings in 15 which:

Fig. 1 is a conventional view partly in elevation and partly in cross section of a wire reducing plant by means of which my process for reducing the cross section of 20 wires and providing them with a roughened surface may be carried out.

Fig. 2 is a plan view thereof.

Fig. 3 is a section on line 3—3 of Fig. 2.

Fig. 4 is a section on line 4—4 of Fig. 2.

25 Referring to the drawings, W is a composite or alloy wire of the material above described reduced to a comparatively large cross section by any known wire working process. 10 is a spool of wire which has reached the limit of its tensile strength by 30 the ordinary wire drawing processes, which spool is placed on a spool holder 12 and so mounted that a suitable tension may be imparted to the wire by various well known means, such as the small weight 14 secured by means of a strap 16 to the holder at 18, said strap passing around a small brake or friction pulley 20. The wire W then passes entirely around a wheel 22 in the direction of 35 the arrow so that the lengths of wire measured by the circumference of the disc or wheel 22 will be recorded when the striker arm 24 engages the arm 26 of a counter mechanism 28 suitably placed upon the pedestal 30.

40 Supported on legs 34 and 36 is a hard rubber receptacle 40, the cavity of which is filled with a suitable electrolyte 42 and which is provided at each end with slots 44 and 46 for the reception of the wire W. The mercury contacts consisting of cylindrical cells 50 and 52 are provided at each end of the hard rubber receptacle 40, the upper parts of the cells being slotted as at 54 and 56 within which 45 the wire also is enabled to pass. As shown, each of these cells is filled with Hg and through each of which the wire is caused to pass. The slots in the cells and in the hard rubber receptacle above referred to while of sufficient width to receive the wire are yet so small that the mercury cannot ooze therefrom, the mercury thus forming a wall against or through which the electrolyte cannot pass. 60 is a copper plate secured at 55 the bottom of the receptacle 40 by means of a

binding post 62, which plate 60 forms the cathode terminal in the electrolyte, the wire acting as the anode. The electric circuit consists of the mercury terminal 50, wire 1, rheostat 2, contact point 3, switch lever 4, wire 5, generator G, wire 6, ammeter A, wire 7, to the binding post 62, thus completing the circuit, the current being so operated that the wire W in the electrolytic bath is the anode and the copper plate 60 is the cathode, as above explained. Adjacent the electrolytic bath is a cleaning tank supported upon suitable supports 37 and 39, as shown, which consists of a copper tube or box 41 being also provided at each end with mercury contacts 61 and 63, slotted as above described at 66 and 68, the slots being of sufficient width to permit the passage of the wire yet prevent the passage therethrough of the mercury. 75

80 Mounted on a support 70 is a pair of spring pressed fingers 72 and 74 pivoted at 76 around which is a spring 78 operating to hold the fingers together. At the end of the fingers are pads 80 and 82 of felt or the like between which the wire passes to clean 85 or dry it. From the cleaning fingers the wire passes to a receiving spool 84 mounted upon a driven shaft 86 journaled on a support 75, to which is also secured a pulley 88 which is driven by means of a motor M 90 through a drive belt 90. Any suitable well known means such as cams for imparting lateral motion to the spool 84 (not shown) are provided to cause the wire to be smoothly and properly wound thereupon.

95 As will be clearly understood, the apparatus just described is suitable for the operation of my processes and the production of the new products desired. To briefly recapitulate, a spool of wire which has reached the limit of its tensile strength by the ordinary wire drawing processes is placed upon a spool holder and the wire then passes through a suitable electrolyte in the electrolytic cell which latter is provided 105 with the mercury contacts as described acting as one terminal, and with a copper contact acting as the other terminal. The wire is subjected to an electrolysis in this cell and being the anode is thus reduced in diameter 110 and is provided with a roughened surface. The wire then passes to a second receptacle filled with water to wash off any chemicals that may have adhered to the wire, and from there passes to the cleaning instrument, as 115 described, and is wound upon the receiving spool by means of the motor, as clearly shown and described. The process is repeated again and again until the wire reaches the desired cross section.

120 I am enabled to reduce the diameter of the wire by a small and uniform amount during each passage of the wire through the electrolyte by causing the wire to pass through the electrolyte at a continuous and 125

uniform speed and regulating the strength of the current in the manner above described.

When tungsten or molybdenum alloys or mixtures are to be acted upon the electrolyte which I have found preferable for use, and which produces excellent results, is prepared by adding to a liter of distilled water 400 gms. to 500 gms. of caustic soda and 10 200 gms. to 250 gms. of potassium ferro-cyanide. Although this electrolyte produces excellent results, it is, of course, obvious that any suitable electrolyte may be used in carrying out my process.

15 When wires of other metals are to be reduced in cross section, I use the standard acid or alkali solutions which are used for the electrolysis of the particular metal under treatment, all of which are well known in 20 the electro-chemical art.

Having thus described my invention what I claim as new and desire to secure by Letters Patent is:

1. The process of producing fine metallic 25 or alloy wires by electro-chemical action which consists in repeatedly passing the wire through an electrolytic bath when immersed in the electrolyte thereof.

2. The process of producing metallic 30 wires which consists in gradually reducing the cross section of said wires by repeatedly drawing the same through the electrolyte in an electrolytic cell.

3. The process of producing wires of fine 35 cross section and of high electron emission by electro-chemical action by repeatedly drawing the wire through the electrolyte of an electrolytic cell.

4. The process of producing wires of fine

cross section and with roughened surface 40 having a high electron emission by reducing the cross section and roughening the surface by repeatedly passing said wire through an electrolyte in an electrolytic cell.

5. In the manufacture of radio tube wire 45 the step of reducing the diameter of said wire by drawing the wire through an electrolyte in an electrolytic cell.

6. In the manufacture of radio tube wire, the steps of repeatedly drawing the wire 50 through a bath of ferro-cyanide and caustic soda.

7. Apparatus of the type described which comprises, a receptacle, mercury pockets in opposing walls of said receptacle, said walls being provided with passageways therethrough into said receptacle to permit the movement of a wire into said receptacle, an electrolyte in said receptacle, the passageways being sufficiently narrow to prevent 60 the escape of mercury from said pockets, the mercury in said pockets forming a seal for the electrolyte, an electric terminal in the receptacle and an electric circuit connection between the mercury and the said terminal. 65

8. Apparatus of the type described which comprises, a receptacle adapted to hold a liquid, mercury pockets in opposite walls of said receptacle the walls of said pockets having passages therethrough leading into 70 and from said receptacle to permit the free movement of a wire through said passages into and from said receptacle, said passages being sufficiently narrow to prevent the escape of mercury from said pockets, the mercury forming seals for the liquid in the receptacle. 75

CLEMENS A. LAISE.